# EUROPEAN PATENT SPECIFICATION

(11) **EP 4 073 302 B1**
(45) Date of publication and mention of the grant of the patent: **11.02.2026**
(21) Application number: 20899270.1
(22) Date of filing: 09.12.2020
(51) Int. Cl.: D06N 7/00, D01F 1/10, D01F 6/62, D02G 3/44, D05C 17/02, D02G 3/04

(54) **COMBINATION YARN**
KOMBINATIONSGARN
FIL COMBINÉ

(30) Priority: 10.12.2019 US 201962946163 P; 31.01.2020 EP 20154782
(43) Date of publication of application: 19.10.2022
(73) Proprietor: Aladdin Manufacturing Corporation, Calhoun, GA 30701 (US)
(72) Inventor: NORTH, Melissa, Adairsville, Georgia 30103 (US); BEASON, Wayne, Dalton, Georgia 30721 (US); CASCIO, Anthony, Calhoun, Georgia 30701 (US)
(74) Representative: Unilin Technologies
(86) International application number: PCT/US2020/063929
(87) International publication number: WO 2021/119076

(56) References cited:
- WO-A1-01/10929
- WO-A2-2012/012597
- JP-A- 2005 023 495
- US-A1- 2001 055 683
- US-A1- 2005 269 439
- US-A1- 2009 013 662
- US-A1- 2009 036 613
- US-A1- 2012 180 232
- US-A1- 2012 282 431
- US-A1- 2015 252 494
- YANG Y ET AL: "DYEING OF PTT/PET BLENDS", AATCC REVIEW,, vol. 2, no. 8, 1 August 2002 (2002-08-01), pages 54 - 59, XP001225386, ISSN: 1532-8813

## Description

### TECHNICAL FIELD

This disclosure relates to combination yarns, and more particularly to polyester yarns and carpets using such yarns as pile yarn.

### BACKGROUND

Carpets, rugs, and mats used in home or commercial applications are typically made from natural fibers (such as cotton or wool) or synthetic fibers (such as nylon, polyester, polyolefins, acrylics, rayon, and cellulose acetate). Synthetic fibers tend to be more favored in carpet manufacture as they are generally more commercially acceptable and can be used for a wider variety of applications.

Nylon is often used in carpet fiber since it is strong, easy to dye, and readily available. Nylon carpeting can be disadvantageous, however, as it generally requires various treatments due to its susceptibility to developing static electric charges and its ease of staining. Carpets made from polyolefins, such as polypropylene, are very resistant to staining and are naturally antistatic; however, polypropylene is a more rigid and less resilient fiber and will not generally maintain its appearance or shape under prolonged or heavy use, or after repeated deformations.

Polyesters such a PET, PTT, and PBT are a favorable alternative to both nylon and polyolefins and are known to provide stain resistance and static resistance while also providing a "wool-like" feel with good physical performance.

WO 2012/012597 A2 relates to polyester yarns made from two or more different polyesters. The invention is also directed to finished articles made from two or more different polyesters, and especially to carpets.

JP 2005 023495 A provides a doubled and twisted yarn for forming a carpet that has both aesthetic appearance of the pencil point-like pattern and high cushioning properties with soft feeling and compression recovery, light resistance, antifouling properties, and provide the carpet by using the doubled and twisted yarn.

### SUMMARY

The present invention is described in claim 1, whereas preferred embodiments of the invention are provided in the dependent claims.

The present disclosure provides combination yarns, in particular combination yarns formed from two or more polyester yarns having different polymeric compositions yet having substantially the same color strength when dyed under the same dyeing conditions, for example when both yarns are dyed together. In other embodiments, the present disclosure provides combinations yarns formed from two or more polyester yarns having different polymeric compositions that provide substantially different color strength between the two yarns when dyed under the same dyeing conditions, for example when both yarns are dyed together.

According to the invention, a combination yarn is provided comprising a first single yarn and a second single yarn, wherein the first single yarn and the second single yarn are linked to each other, wherein the first single yarn comprises at least 60% polyethylene terephthalate (PET), wherein the second single yarn comprises at least 60% polytrimethylene terephthalate (PTT), and wherein at least one of the first single yarn and the second single yarn includes one or more additives that increase dye uptake of disperse dyes or solution dyes such that the color strength of the at least one of the first single yarn and the second single yarn is increased when compared to the same first single yarn and/or the same second single yarn which does not include the one or more additives.

In some embodiments, the first single yarn includes the one or more additives. In some embodiments where the first single yarn includes the one or more additives, the second single yarn does not include the one or more additives. In some embodiments where the first single yarn includes the one or more additives, the color strength of the first single yarn is within 20% or within 10% of the color strength of the second single yarn when both yarns are subjected to the same dyeing conditions, for example when both yarns are dyed together.

In some embodiments, the second single yarn includes the one or more additives. In some embodiments where the second single yarn includes the one or more additives, the first single yarn does not include the one or more additives. In other embodiments where the second single yarn includes the one or more additives, the first single yarn also includes the one or more additives. In some embodiments where both the first and the second single yarn include the one or more additives, the one or more additives included with the first single yarn are different from the one or more additives included with the second single yarn. In some embodiments where the second single yarn includes the one or more additives, the color strength of the second single yarn is at least 10% or at least 20% greater than the color strength of the first single yarn when both yarns are subjected to the same dyeing conditions, for example when both yarns are dyed together.

In one aspect, according to the invention, a combination yarn is provided comprising a first single yarn and a second single yarn, wherein the first single yarn and the second single yarn are linked to each other, wherein the first single yarn comprises polyethylene terephthalate (PET) and at least one or more additives which increase dye uptake of disperse dyes or solution dyes, wherein the second single yarn comprises polytrimethylene terephthalate (PTT) and does not include one or more additives which increase dye uptake, and wherein the color strength of the first single yarn is within 20% or within 10% of the color strength of the second single yarn when both yarns are subjected to the same dyeing conditions, for example, when both yarns are dyed together. In some embodiments, the first single yarn comprises at least 75% PET. In some embodiments, the second single yarn comprises at least 75% PTT.

In another aspect, according to the invention, a combination yarn is provided comprising a first single yarn and a second single yarn, wherein the first single yarn and the second single yarn are linked to each other, wherein the first single yarn comprises PET, wherein the second single yarn comprises PTT and one or more additives which increase dye uptake of disperse dyes or solution dyes, and wherein the color strength of the second single yarn is at least 10% or at least 20% greater than the color strength of the first single yarn when both yarns are subjected to the same dyeing conditions, for example when both yarns are dyed together. In some embodiments, the first single yarn does not include one or more additives which increase dye uptake. In other embodiments, the first single yarn does include one or more additives which increase uptake, wherein the one or more additives for the first single yarn may be the same or different from the one or more additives for the second single yarn.

In some embodiments, the one or more additives that increase dye uptake may include polybutylene terephthalate (PBT), at least one ester modifier, or combinations thereof. In some embodiments, the ester modifier includes a copolymer formed by polymerization of a mixture comprising terephthalic acid or esters thereof, at least one dicarboxylic acid monomer, and at least one diol monomer. In other embodiments, the ester modifier includes a copolymer formed by polymerization of a mixture comprising terephthalic acid or esters thereof, at least one diol monomer, and at least one polyalkylene glycol. In some embodiments, the ester modifier includes ortho-phthalic acid, isophthalic acid, esters thereof, or mixtures thereof.

In some embodiments, the first single yarn and/or the second single yarn are continuous filament yarns. Each of the first single yarn and the second single yarn may comprise a given number of filaments per cross section, which number of filaments per cross section may be identical or different for the first single yarn and second single yarn.

In some embodiments, all filaments of the first single yarn may have a substantially equal cross section. In some embodiments, all filaments of the second single yarn may have a substantially equal cross section. In some embodiments, the cross sections of the filaments of the first single yarn and the second single yarn may be substantially identical (having cross-sectional areas within 10% of each other).

In some embodiments, the first single yarn or the second single yarn are bulked continuous filament (BCF) yarns. In other embodiments, the first single yarn or the second single yarn are spun yarns comprising staple fibers.

In some embodiments, the combination yarn may be a plied or twisted yarn. The combination yarn may be plied or twined in either the S- or Z-direction. The first single yarn, second single yarn, or further single yarns may be untwisted, particularly when the single yarns are BCF yarns, or may be twisted as well.

The use of the combination yarn as described herein as a pile yarn in a carpet is also provided. In some embodiments, the carpet is a tufted carpet.

Also provided is a tufted carpet comprising a pile yarn providing the pile of the carpet, wherein the pile yarn is the combination yarn described herein.

The details of one or more embodiments of the disclosure are set forth in the description below. Other features, objects, and advantages of the disclosure will be apparent from the description and from the claims.

### DETAILED DESCRIPTION

In one aspect, a combination yarn is provided comprising a first single yarn and a second single yarn, wherein the first single yarn and second single yarn are linked to each other, wherein the first single yarn comprises primarily polyethylene terephthalate (PET), and wherein the second single yarn comprises primarily polytrimethylene terephthalate (PTT). In some embodiments, the color strength of the first single yarn is within 20%, within 15%, within 10%, or within 5% of the color strength of the second single yarn when both yarns are subjected to the same dyeing conditions. In other embodiments, the color strength of the second single yarn is at least 10%, at least 20%, or at least 30% greater than the color strength of the first single yarn when both yarns are subjected to the same dyeing conditions. In some embodiments, the first single yarn and second single yarn are subjected to dyeing together.

The first single yarn may comprise filaments or fibers, which filaments or fibers are made primarily from polyethylene terephthalate (PET) and hence comprise at least 60% PET, and may further include common additives like process enhancers, stabilizers, fillers, and the like. In some embodiments, the PET as used in the first single yarn may originate from recycled PET products such as recycled PET bottles, also referred to as rPET. The first single yarn includes at least 60%, preferably at least 70%, more preferably at least 75%, more preferably at least 80%, more preferably at least 90%, more preferably at least 95%, or even more preferably at least 99% PET.

The second single yarn may comprise filaments or fibers, which filaments or fibers are made primarily from polytrimethylene terephthalate (PTT) and hence comprise at least 60% PTT as the majority of the material, and may further include common additives like process enhancers, stabilizers, fillers and the like. In some embodiments, the PTT as used in the second single yarn may originate from recycled PTT products, also referred to as rPTT. The second single yarn includes at least 60%, preferably at least 70%, more preferably at least 75%, more preferably at least 80%, more preferably at least 90%, more preferably at least 95%, or even more preferably at least 99% PTT.

The combination yarn may have a linear weight, expressed in dtex, in the range of 1111 to 1778 dtex (1000 to 1600 denier), more preferably 1222 to 1667 dtex (1100 to 1500 denier). A 'denier' equals one gram per 9000 meters of yarn. Either the first single yarn or the second single yarn may have a linear weight, expressed dtex, in the range of 556 to 889 dtex (500 to 800 denier), more preferably 611 to 833 dtex (550 to 750 denier). In some embodiments, the first single yarn and the second single yarn, and if present also any further single yarn, have substantially equal linear weights (within 10% of each other).

In some embodiments, the first single yarn and/or the second single yarn are continuous filament yarns. Each of the first single yarn and the second single yarn may comprise a given number of filaments per cross section, which number of filaments per cross section may be identical or different for the first single yarn and second single yarn. The number of filaments may be between 120 and 160, preferably between 123 and 150. Each filament has a thickness, in function as an element of the yarn, typically expressed as "denier per filament" or "dpf." The filaments of the first single and/or second single yarn may have a thickness in the range of 11.1 to 13.3 dtex per filament (10 to 12 dpf), more preferably in the range of 11.6 to 12.4 dtex per filamant (10.4 to 11.2 dpf). Thus, each filament of the first single yarn and the second single yarn may have a thickness in the range of 11.1 to 13.3 dtex per filament (10 to 12 denier), more preferably in the range of 11.6 to 12.4 dtex per filament (10.4 to 11.2 denier).

Each filament of the first and second single yarn has a cross section which may be circular, oval, triangular, trilobal, or square. Optionally, the filaments may be hollow, comprising one or a plurality of hollow channels. These one or more channels may be coaxial with the axis of the filament.

In some embodiments, all filaments of the first single yarn may have a substantially equal cross section with a cross-sectional area within 10% of the mean cross-section. In some embodiments, all filaments of the second single yarn may have a substantially equal cross section with a cross-sectional area within 10% of the mean cross-section. In some embodiments, the mean cross-section of the filaments of the first single yarn and the mean cross-section of the filaments in the second single yarn are substantially identical, i.e., within 10% of each other.

In some embodiments, the first single yarn or the second single yarn are bulked continuous filament (BCF) yarns. In other embodiments, the first single yarn or the second single yarn are spun yarns comprising staple fibers.

In some embodiments, the first single yarn is a primarily PET single yarn as discussed herein including one or more additives that increase dye uptake. In other embodiments, the second single yarn is a primarily PTT single yarn as described herein including one or more additives that increase dye uptake. In yet other embodiments, both the first single yarn and the second single yarn as described herein include one or more additives that increase dye uptake. In some embodiments, an increase in dye uptake is defined by an increase in color strength for the first single yarn or the second single yarn, as measured by colorimetry, of 20% or more as compared to a control first single yarn or a control second single yarn respectively that does not contain the one or more additives that increase dye uptake when exposed to the same dyeing conditions. In some embodiments, the first single yarn or the second single yarn shows a greater than 20%, greater than 40%, greater than 60%, greater than 80%, greater than 100%, greater than 150%, greater than 200%, greater than 250%, greater than 300%, or greater than 400% increase in color strength, as compared to a control first single yarn or a control second single yarn that does not contain the one or more additives that increase dye uptake, when exposed to the same dyeing conditions.

"Color Strength" as used herein refers to the ability of a pigment or dye to change the color of an otherwise colorless material. Color strength may be measured, for example, by comparing the K/S value (where K represents the absorbance and S represents the scatter of the material) of a material, such as the first single yarn or the second single yarn described herein, to a known standard, for example a control first single yarn or a control second single yarn respectively that does not contain one or more additives that increase dye uptake, when exposed to the same dyeing conditions. In some embodiments, the K/S value may be measured from the reflectance of the dyed material as determined by Kubelka-Monk theory using the following formula: K/S = [{(1-R)²/2R)]. Thus, in some embodiments, the first single yarn or the second single yarn as described herein shows an increase in its K/S value of 20% or more as compared to the K/S value of the control first single yarn or the control second single yarn, respectively. In some embodiments, the first single yarn or the second single yarn as described herein shows a 20% or greater, 40% or greater , 60% or greater, 80% or greater, 100% of greater, 150% or greater, 200% or greater, 250% or greater, 300% or greater, or 400% or greater increase in its K/S value as compared to the K/S value of the control first single yarn or the control second single yarn, respectively. K/S values may be measured using any number of commercially available spectrophotometers, for example, the Datacolor^{®} 800 spectrophotometer.

Whether the first single yarn, the second single yarn, or both further include one or more additives that increase dye uptake depends on the desired color strength difference between the two single yarns for the particular desired application. In some embodiments, the color strength of the first single yarn is desired to be within 20% or within 10% of the color strength of the second single yarn when both are subjected to the same dyeing conditions. In these embodiments, the first single yarn comprises primarily PET and one or more additives that increase dye uptake and the second single yarn comprises primarily PTT and does not include any additives that increase dye uptake. Such embodiments typically are directed to applications where uniformity of color is desired, such as unicolor carpets. In other embodiments, the color strength of the second single yarn is instead desired to be at least 10% or at least 20% greater than the color strength of the first single yarn when both yarns are subjected to the same dyeing conditions. In these embodiments, both the first single yarn and the second single yarn may further comprise one or more additives to increase dye uptake, or the second single yarn may further comprise one or more additives to increase dye uptake while the first single yarn does not include one or more of such additives.

In some embodiments, the one or more additives that increase dye uptake may include polybutylene terephthalate (PBT), at least one ester modifier, or combinations thereof. In some embodiments, the one or more additives that increase dye uptake include polybutylene terephthalate (PBT). In some embodiments, the one or more additives that increase dye uptake include at least one ester modifier. In other embodiments, the one or more additives that increase dye uptake include both polybutylene terephthalate (PBT) and at least one ester modifier. In some embodiments, polybutylene terephthalate (PBT) can be present in an amount from 2.5 wt. % to 12 wt. %, from 3 wt. % to 12 wt. %, from 4 wt. % to 11 wt. %, from 5 wt. % to 10 wt. %, from 5.5 wt. % to 9.5 wt. %, or from 6 wt. % to 8 wt. % based on the total polymer weight of the first or second single yarn. In some embodiments, PBT can be present at 2.5 wt. %, 3 wt. %, 4 wt. %, 5 wt. %, 6 wt. %, 7 wt. %, 8 wt. %, 9 wt. %, 10 wt. %, 11 wt. %, or 12 wt. % based on the total polymer weight of the first or second single yarn. In one embodiment, PBT is present at 7.5 wt. % based on the total polymer weight of the first or second single yarn. In some embodiments, the ester modifier can be present in an amount ranging from 2.5 wt. % to 12 wt. %, from 3 wt. % to 10 wt. %, from 4 wt. % to 8 wt. %, from 5 wt. % to 7 wt. %, or from 5.5 wt. % to 6.5 wt. % based on the total polymer weight of the first or second single yarn. In some embodiments, the ester modifier can be present at 2.5 wt. %, 3 wt. %, 4 wt. %, 5 wt. %, 6 wt. %, 7 wt. %, 8 wt. %, 9 wt. %, 10 wt. %, 11 wt. %, or 12 wt. % based on the total polymer weight of the first or second single yarn. In one embodiment, the ester modifier is present at 6 wt. % based on the total polymer weight of the first or second single yarn. In another embodiment, the ester modifier is present at 8 wt. % based on the total polymer weight of the first or second single yarn.

Ester modifiers may typically comprise compounds that chemically modify the polyester such that it has decreased crystallinity. This decrease in crystallinity provides more space for the dye to penetrate the polymer matrix formed from the polyester, resulting in an increase in dye uptake.

In some embodiments, the ester modifier comprises a copolymer formed by polymerization of a mixture comprising terephthalic acid or esters thereof, at least one dicarboxylic acid monomer, and at least one diol monomer. In other embodiments, the ester modifier comprises a copolymer formed by polymerization of a mixture comprising terephthalic acid or esters thereof, at least one diol monomer, and at least one polyalkylene glycol. In one embodiment, the mixture comprises terephthalic acid or an ester thereof, a diol monomer, and a dicarboxylic acid monomer in a ratio of 1:2:1. In one embodiment, the mixture includes terephthalic acid. In one embodiment, the mixture includes dimethyl terephthalate.

In some embodiments, the at least one dicarboxylic acid monomer can be selected from an aliphatic and/or aromatic acid. In some embodiments, the at least one dicarboxylic acid monomer can be selected from isophthalic acid, 2,6-naphthalene dicarboxylic acid, 3,4'-diphenyl ether dicarboxylic acid, hexahydrophthalic acid, 2,7-naphthalenedicarboxylic acid, phthalic acid, 4,4'-methylenebis(benzoic acid), oxalic acid, malonic acid, succinic acid, methyl succinic acid, glutaric acid, adipic acid, 3-methyladipic acid, pimelic acid, suberic acid, azelaic acid, sebacic acid, 1,11-undecanedicarboxylic acid, 1,10-dodecanedicarboxylic acid, undecanedioic acid, 1,12-dodecanedicarboxylic acid, hexadecanedioic acid, docosanedioic acid, tetracosanedioic acid, 1,4-cyclohexanedicarboxylic acid, 1,3-cyclohexanedicarboxylic acid, 1,2-cyclohexanediacetic acid, fumaric acid, maleic acid, or combinations thereof. In some embodiments, the at least one dicarboxylic acid is selected from succinic acid, glutaric acid, adipic acid, sebacic acid, or combinations thereof. In one embodiment, the dicarboxylic acid monomer is adipic acid.

In some embodiments, the at least one diol monomer can be selected from an aliphatic diol, a cyclic diol, and/or an aromatic diol. In some embodiments, the at least one diol can be selected from monoethylene glycol, diethylene glycol, triethyleneglycol, poly(ethylene ether)glycols, 1,3-propanediol, 1,4-butanediol, poly(butylene ether)glycols, 1,6-hexanediol, 1,8-octanediol, 1,10-decanediol, 1,12-dodecanediol, 1,14-tetradecanediol, 1,16-hexadecanediol, and cis- or trans-1,4-cyclohexanedimethanol. In some embodiments, the diol is selected from ethylene glycol, 1,3-propanediol, and 1,4-butanediol. In other embodiments, the diol can be selected from 1,4-butanediol, 1,5-pentanediol, or 1,6-hexanediol. In one embodiment, the diol includes 1,4-butanediol.

In some embodiments, the polyalkylene glycol can be selected from the group consisting of polyethylene glycol, polypropylene glycol, ethylene oxide-propylene oxide copolymers, or combinations thereof. In some embodiments, the polyalkylene glycol includes polyethylene glycol. In some embodiments, the polyethylene glycol has a molecular weight from 200 to 5000 g/mol.

In some embodiments, the mixture further comprises sodium dimethyl-5-sulfoisophthalate (DMSIP), 5-sulfoisophthalic acid (SIPA), or combinations thereof. In some embodiments, the mixture includes dimethyl-5-sulfoisophthalate (DMSIP). In some embodiments, the mixture includes 5-sulfoisophthalic acid.

In some embodiments, the ester modifier comprises polybutylene adipate terephthalate (PBAT).

In some embodiments, the mixture further comprises a chain extender. In some embodiments, the chain extender can be selected from compounds comprising at least three groups capable of ester formation, for example but not limited to: tartaric acid, citric acid, malic acid, trimethylolpropane, trimethylolethane, pentaerythritol, polyether triols, glycerol, trimesic acid, trimellitic acid, trimellitic anhydride, pyromellitic acid, pyromellitic dianhydride and hydroxyisophthalic acid. In other embodiments, the chain extender is selected from compound comprising at least two isocyanate groups, for example but not limited to: aromatic isocyanates including tolylene 2,4-diisocyanate, tolylene 2,6-diisocyanate, 2,2'-diphenylmethane diisocyanate, 2,4'-diphenylmethane diisocyanate, 4,4'-diphenylmethane diisocyanate, naphthylene 1,5-diisocyanate, or xylylene diisocyanate; aliphatic diisocyanates such as 1,6-hexamethylene diisocyanate, isophorone diisocyanate, and methylenebis(4-isocyanatocyclohexane); trinuclear isocyanates such as tri(4-isocyanophenyl)methane; and isocyanurates derived from aliphatic isocyanates such as isophorone diisocyanate or methylenebis(4-isocyanatocyclohexane).

In other embodiments, the ester modifier may be selected from a phthalate plasticizer. Representative examples of phthalate plasticizers as can be used in the present invention include, but are not limited to, bis(2-ethylhexyl)phthalate (DEHP), bis(2-propylheptyl)phthalate (DPHP), diisononyl phthalate (DINP), di-n-butyl phthalate (DnBP), butyl benzyl phthalate (BBzP), diisodecyl phthalate (DIDP), dioctyl phthalate (DOP), diisooctyl phthalate (DIOP), diethyl phthalate (DEP), diisobutyl phthalate (DIBP), and di-n-hexyl phthalate. In some embodiments, the ester modifier may be selected from ortho-phthalic acid, isophthalic acid, or esters thereof.

In some embodiments, the PET as used in the first single yarn described herein can further comprise one or more additional monomeric or polymeric units. In one particular embodiment, the one or more additional monomeric units comprises cyclohexane dimethanol (CHDM), wherein a PET polymer including a percentage of CHDM may also be known as PETG. In some embodiments, the one or more additional units can comprise one or more isophthalic acids, including sulfonated isophthalic acids. In some embodiments, the one or more additional units can be selected from diethylene glycol, polyethylene glycol, butylene glycol, polystyrene, vinyltoluene, halostyrene, dihalostyrene, styrene-butadiene copolymers, styrene-acrylonitrile copolymers, styrene-acrylonitrile-butadiene copolymers, styrene-butadiene-styrene terpolymers, styrene-isoprene copolymers, aromatic dicarboxylic acids such a 5-sodium sulfoisophthalic acid, aliphatic dicarboxylic acids such as adipic acid and itaconic acid, glutaric acid, azelaic acid, sebacic acid, and combinations thereof. In some embodiments, the one or more additional units can comprise branching agents such as trimesic acid, pyromellitic acid, trimethylolpropane, trimethylolethane, and pentaerythritol.

In some embodiments, the PTT as used in the second single yarn described herein can further comprise one or more additional monomeric units. Representative examples of the additional monomeric units include 5-sodium sulfoisophthalic acid, 5-potassium sulfoisophthalic acid, 4-sodium sulfo-2,6-naphthalenedicarboxylate, tetramethylphosphonium-3,5-dicarboxybenzenesulfonate, tetrabutylphosphonium 3,5-dicarboxybenzenesulfonate, tributylmethylphosphonium 3,5-dicarboxybenzenesulfonate, tetrabutylphosphonium 2,6-dicarboxynaphthalene-4-sulfonate, tetramethylphosphonium 2,6-dicarboxynaphthalene-4-sulfonate, ammonium 3,5-dicarboxybenzenesulfonate, 1,2-butanediol, 1,3-butanediol, 1,4-butanediol, neopentyl glycol, 1,5-pentamethylene glycol, 1,6-hexamethylene glycol, heptamethylene glycol, octamethylene glycol, decamethylene glycol, dodecamethylene glycol, 1,4-cyclohexanediol, 1,3-cyclohexanediol, 1,2-cyclohexanediol, 1,4-cyclohexanedimethanol, 1,3-cyclohexanedimethanol, 1,2-cyclohexanedimethanol, oxalic acid, malonic acid, succinic acid, glutaric acid, adipic acid, heptanedioic acid, octanedioic acid, sebacic acid, dodecanedioic acid, 2-methylglutaric acid, 2-methyladipic acid, fumaric acid, maleic acid, itaconic acid, 1,4-cyclohexanedicarboxylic acid, 1,3-cyclohexanedicarboxylic acid, and 1,2-cyclohexanedicarboxylic acid.

In some embodiments, the yarns as described herein may comprise one or more further additives, including but not limited to: flame retardant additives, for example decabromodiphenyl ether and triaryl phosphates such as triphenyl phosphate; reinforcing agents such as glass fibers; thermal stabilizers, for example thermal conductivity improves such as zinc oxide and titanium oxide; ultraviolet light stabilizers such as resorcinol monobenzoates, phenyl salicyclate and 2-hydroxybenzophenones; hindered amine stabilizers such as benzotriazole, benzophenone, oxalanilide, and cerium oxide; impact modifiers; flow enhancing additives; ionomers; liquid crystal polymers; fluoropolymers; olefins including cyclic olefins; polyamides; ethylene vinyl acetate copolymers; stabilizing agents such as ortho-phosphoric acid, trimethyl phosphate, triphenylphosphate, and triethylphosphino acetate; delustering agents such as titanium oxide; carriers such as o-phenylphenol, p-phenylphenol, o-dichlorobenzene, trichlorobenzene, monochlorobenzene, biphenyl, methyl salicyclate, butyl benzoate, benzyl benzoate, benzoic acid, benzalacetone, and methyl cinnamate; leveling agents such as asbishydroxymethyloxazoline, diaryl ethers, ditolyl ether, sodium di-naphthylmethane-B,B disulfonate, ammonium dodecylbenzene sulfonate, sodium tetrapropylbenzene sulfonate, homopolymers or oligomers of N-vinyl pyrrolidone or poly tetrahydrofuran; and porosity additives such as metal oxalate complexes, organic sulfonate salts, jade powder, or zeolite powder.

In an embodiment of the invention, a combination yarn is provided comprising a first single yarn and a second single yarn,
wherein the first single yarn and the second single yarn are linked to each other,
wherein the first single yarn comprises at least 60% (for example, at least 75%) PET and an additive that includes at least one ester modifier,
wherein the second single yarn comprises at least 60% (for example, at least 75%) PTT and does not include any additives that increase dye uptake, and
wherein the color strength of the first single yarn is within 20% (for example, within 10%) of the color strength of the second single yarn when both yarns are subject to the same dyeing conditions, for example, when both yarns are dyed together.

In an embodiment of the invention, a combination yarn is provided comprising a first single yarn and a second single yarn,
wherein the first single yarn and the second single yarn are linked to each other,
wherein the first single yarn comprises at least 60% (for example, at least 75%) PET and does not include any additives that increase dye uptake,
wherein the second single yarn comprises at least 60% (for example, at least 95%) PTT and an additive that includes PBT and at least one ester modifier, and
wherein the color strength of the second single yarn is at least 10% (for example, at least 20%) greater than the color strength of the first single yarn when both yarns are subject to the same dyeing conditions, for example when both yarns are dyed together.

A disperse dye may be used to color the first single yarn and/or the second single yarn. In some embodiments, the same disperse dye may be used to color the first single yarn and the second single yarn. For example, the first single yarn and the second single yarn may be dyed together. In other embodiments, the first single yarn and the second single yarn may be dyed to the same or to a different dye tone using the same disperse dye.

In some embodiments, a combination yarn is provided comprising at least a first single yarn and a second single yarn, wherein the first single yarn is a polyethylene terephthalate (PET) single yarn, wherein the second single yarn is a polytrimethylene terephthalate (PTT) single yarn, and wherein the first single yarn and/or the second single yarn have been solution dyed. For example, the first single yarn and the second single yarn may be dyed together.

The combination yarn as described herein may be dyed using a piece dyeing process. In a piece dyeing process, the undyed combination yarn is first assembled as a component of the final object, for example as pile fibers in a carpet. The assembled final object, for example a carpet, is then immersed in a dye bath at an elevated temperature. Depending upon the composition of the first single yarn and the second single yarn of the combination yarn described herein, the final object such as a carpet may be unicolor or may be subject to a differential or tonal effect due to different dyeing levels for the first and second single yarns. In some embodiments, the piece dyeing process may be a continuous dyeing process, where the final objected is passed under dyeing equipment that flows dye solution through the object instead of requiring immersion within a dye bath.

In some embodiments, the first single yarn and the second single yarn are dyed at the same temperature. For example, the first single yarn and the second single yarn can be dyed at a temperature less than 135 °C, for example at a temperature of from 100°C to 130°C.

In some embodiments, the first single yarn and the second single yarn may be linked by being formed into a plied or twisted yarn. The combination yarn may be plied or twined in either the S- or Z-direction. The number of turns per centimeter may be in the range of 1.61 to 1.69 turns. (The number of turns per inch may be in the range of 4.10 to 4.30 turns.) In some embodiments, the number of turns per centimeter may be in the range of 1.65 to 1.67 turns. (In some embodiments, the number of turns per inch may be in the range of 4.20 to 4.25 turns.)

The first single yarn, second single yarn, or further single yarns may be untwisted, particularly when the single yarns are BCF yarns, or may be twisted as well. In some embodiments, the twisted single yarn is twisted in a direction (S- or Z-direction) which is opposite to the twining or plying direction. In some embodiments, the twisted single yarn may be twisted in the range of 1.61 to 1.69 turns per centimeter. (In some embodiments, the twisted single yarn may be twisted in the range of 4.10 to 4.30 turns per inch.) In some embodiments, the twisted single yarn may be twisted by 1.67 turns per centimeter. (In some embodiments, the twisted single yarn may be twisted by 4.25 turns per inch.)

In some embodiments, the first single yarn and the second single yarn are linked to each other by air entanglement.

In some embodiments, the combination yarn may comprise more than two single yarns, such as 3, 4, 5 or more single yarns all linked to each other as described herein. In embodiments containing 3 or more single yarns, the additional single yarns may be PET single yarns or PTT single yarns. Depending upon the number of single yarns the properties of the filaments or fibers used to provide the single yarns, the weight ratio of PET to PTT in the combination yarn may vary. In some embodiments, the combination yarn may have a weight ratio of PET to PTT between 4:1 to 1:4. In some embodiments, the combination yarn may have a weight ratio of PET to PTT of 1:1.

In some embodiments, the combination yarn is heat set. In some embodiments, the combined yarn is heat set through, e.g., a Suessen or Superba heat set tunnel, thereby imposing at least to some extent memory, strength and wearability to the yarn.

The combination yarns described herein have several advantages over prior PET-based yarns, particularly when used to provide the pile of a woven or tufted carpet. The addition of PTT yarns to PET-based carpet brings durability, wear and stain resistance with only a portion of the PET yarns being replaced by PTT.

Thus, use of the combination yarn of the invention as a pile yarn in a carpet is also provided. In some embodiments, the carpet is a tufted carpet.

Also provided is a tufted carpet comprising a pile yarn providing the pile of the carpet, wherein the pile yarn is the combination yarn described herein. In some embodiments, the tufted carpet may be provided from solely polyester material, i.e., all parts of the carpet, such as pile yarn, primary backing in which the pile is tufted, the adhesion layer to lock the pile in the primary backing, the secondary backing and the like are provided from a polyester material. In some embodiments, the polyester material is only PET or PTT.

In some embodiments, the carpet is a unicolor carpet. A unicolor carpet is defined by having all the yarns providing the pile of the carpet having a substantially uniform color over the surface of the carpet.

In other embodiments, the carpets may instead have a tonal effect to differing coloration of the first single yarn and the second single yarn. In some embodiments, the carpet is initially assembled as a greige roll, i.e. a roll of the tufted undyed combination yarn without a secondary backing. This greige roll may then be subjected to a piece dyeing process as described herein by immersion into a dye bath or by a continuous dyeing process.

In some embodiments, the carpet may be a loop pile carpet. In other embodiments, the carpet may be a cut pile carpet. In yet other embodiments, the carpet may comprise both cut piles and loop piles.

In some embodiments, the surface weight of the carpet may vary between 847.6 gsm and 2034.3 gsm (25 and 60 ounces per square yard). The height of the pile of the carpet may be between 0.48 centimeter and 6.53 centimeter, for example between 0.635 to 1.27 centimeter or between 1.27 to 1.905 centimeter. (The height of the pile of the carpet may be between 6/32 inches and 2.5 inches, for example between 1/4 to 1/2 inches or between 1/2 to ¾ inches.) The thickness of the carpet may be between 0.95 centimeter and 2.54 centimeter. (The thickness of the carpet may be between 12/32 of an inch and 1 inch.) The number of tufts or pile units per surface unit may be between 250,000 and 25,000 per square meter. The number of piles or tufts in the production direct per centimeter may be in the range of 2.36 to 5.12. (The number of piles or tufts in the production direct per inch may be in the range of 6 to 13.) The distance between two adjacent tufts (or gauge) may range from 0.48 centimeter to 0.25 centimeter. (The distance between two adjacent tufts (or gauge) may range from 3/16 of an inch to 1/10 of an inch.)

### EXAMPLES

By way of non-limiting illustration, examples of certain embodiments of the present disclosure are given below.

### Example 1 - Combination Yarn I

A first example of a combination yarn according to the present disclosure was provided by plying a first single yarn and a second single yarn, the first single yarn being a polyethylene terephthalate (PET) single yarn comprising 8% of BASF 3S ester modifier and the second single yarn being a polytrimethylene terephthalate (PTT) single yarn.

The first single yarn was a bulk continuous filament yarn formed from 150 PET filaments. Each filament has 11.6 dtex (a denier of 10.4) and has a trilobal cross section, providing a single yarn with 1733 dtex (1560 denier). The PET used includes 92 wt. % PET and 8% BASF 3S Modifier.

The second single yarn was a bulk continuous filament yarn formed from 123 PTT filaments. Each filament has 11.6 dtex (a denier of 10.4) and a trilobal cross section, providing a single yarn with 1421 dtex (1279 denier).

The two single yarns were plied with 1.67 turns per centimeter (4.25 turns per inch) in the S-direction, providing a two-ply combination yarn. The two-ply yarn was heat set using a Superba textured heat set tunnel.

A solid dyeable two-ply combination yarn was provided by the above process with little to no tonal aspect visible to the naked eye upon dyeing. This yarn was used to create a solid color fabric that shows better performance than 100% PET fabrics made of the same construction.

## Claims

1. Combination yarn comprising a first single yarn and a second single yarn,
wherein the first single yarn and the second single yarn are linked to each other,
wherein the first single yarn comprises at least 60% polyethylene terephthalate (PET),
wherein the second single yarn comprises at least 60% polytrimethylene terephthalate (PTT), and
wherein at least one of the first single yarn and the second single yarn includes one or more additives that increase dye uptake of disperse dyes or solution dyes such that the color strength of the at least one of the first single yarn and the second single yarn is increased when compared to the same first single yarn and/or the same second single yarn which does not include the one or more additives.

2. Combination yarn according to claim 1, **characterized in that** the one or more additives includes polybutylene terephthalate (PBT), at least one ester modifier, or combinations thereof.

3. Combination yarn according to claim 2, **characterized in that** the ester modifier comprises a copolymer formed by polymerization of a mixture comprising terephthalic acid or esters thereof, at least one dicarboxylic acid monomer, and at least one diol monomer,
wherein the at least one dicarboxylic acid monomer is selected from an aliphatic and/or aromatic acid, from isophthalic acid, 2,6-naphthalene dicarboxylic acid, 3,4'-diphenyl ether dicarboxylic acid, hexahydrophthalic acid, 2,7-naphthalenedicarboxylic acid, phthalic acid, 4,4'-methylenebis(benzoic acid), oxalic acid, malonic acid, succinic acid, methyl succinic acid, glutaric acid, adipic acid, 3-methyladipic acid, pimelic acid, suberic acid, azelaic acid, sebacic acid, 1,11-undecanedicarboxylic acid, 1,10-dodecanedicarboxylic acid, undecanedioic acid, 1,12-dodecanedicarboxylic acid, hexadecanedioic acid, docosanedioic acid, tetracosanedioic acid, 1,4-cyclohexanedicarboxylic acid, 1,3-cyclohexanedicarboxylic acid, 1,2-cyclohexanediacetic acid, fumaric acid, maleic acid, or combinations thereof, or from succinic acid, glutaric acid, adipic acid, sebacic acid, or combinations thereof, or wherein the at least one dicarboxylic acid monomer is adipic acid; or the ester modifier comprises a copolymer formed by polymerization of a mixture comprising terephthalic acid or esters thereof, at least one diol monomer, and at least one polyalkylene glycol.

4. Combination yarn of claim 2, **characterized in that** the ester modifier is selected from the group consisting of ortho-phthalic acid, isophthalic acid, or esters thereof.

5. Combination yarn according to any of the preceding claims, **characterized in that** the first single yarn comprises at least 75% PET, and/or **in that** the second single yarn comprises at least 75% PTT.

6. Combination yarn according to any of the preceding claims, **characterized in that** the first single yarn and/or the second single yarn is a bulked continuous filament yarn.

7. Combination yarn according to any of the preceding claims, **characterized in that** the weight ratio of PET to PTT in the combination yarn is 1:1 to 1:4.

8. Combination yarn according to any of the preceding claims 1 - 7, **characterized in that** the first single yarn includes the one or more additives, wherein the color strength of the first single yarn is within 20% or within 10% of the color strength of the second single yarn when both yarns are subjected to the same dyeing conditions, wherein the color strength of the at least one of the first single yarn and the second single yarn is expressed by a K/S value where K represents the absorbance and S represents the scatter of the material, said value being determined by a spectrophotometer and/or being calculated from the Kubelka-Monk formula.

9. Combination yarn according to any one of claims 1 - 8,
wherein the first single yarn comprises at least 75% PET and an additive that includes at least one ester modifier,
wherein the second single yarn comprises at least 75% PTT and does not include any additives that increase dye uptake of disperse dyes or solution dyes, and
wherein the color strength of the first single yarn is within 10% of the color strength of the second single yarn when both yarns are subject to the same dyeing conditions,
wherein the color strength of the at least one of the first single yarn and the second single yarn is expressed by a K/S value where K represents the absorbance and S represents the scatter of the material, said value being determined by a spectrophotometer and/or being calculated from the Kubelka-Monk formula.

10. Combination yarn according to any of the preceding claims 1 - 7, **characterized in that** the second single yarn includes the one or more additives, wherein the color strength of the second single yarn is at least 10% or at least 20% greater than the color strength of the first single yarn when both yarns are subjected to the same dyeing conditions, wherein the color strength of the at least one of the first single yarn and the second single yarn is expressed by a K/S value where K represents the absorbance and S represents the scatter of the material, said value being determined by a spectrophotometer and/or being calculated from the Kubelka-Monk formula.

11. Combination yarn according to any one of claims 1 - 7 or 10,
wherein the first single yarn comprising at least 75% PET and does not include any additives that increase dye uptake of disperse dyes or solution dyes,
wherein the second single yarn comprises at least 75% PTT and an additive that includes PBT and at least one ester modifier, and
wherein the color strength of the second single yarn is at least 20% greater than the color strength of the first single yarn when both yarns are subject to the same dyeing conditions,
wherein the color strength of the at least one of the first single yarn and the second single yarn is expressed by a K/S value where K represents the absorbance and S represents the scatter of the material, said value being determined by a spectrophotometer and/or being calculated from the Kubelka-Monk formula.

12. Combination yarn according to any one of claims 1 - 7 or 10,
wherein the first single yarn comprises at least 75% PET,
wherein the second single yarn comprises at least 95% PTT,
wherein both the first single yarn and the second single yarn further comprise an additive that includes PBT, at least one ester modifier, or combinations thereof, and
wherein the color strength of the second single yarn is at least 20% greater than the color strength of the first single yarn when both yarns are subject to the same dyeing conditions,
wherein the color strength of the at least one of the first single yarn and the second single yarn is expressed by a K/S value where K represents the absorbance and S represents the scatter of the material, said value being determined by a spectrophotometer and/or being calculated from the Kubelka-Monk formula.

13. Combination yarn according to any one of the preceding claims excluding claims 9 and 11, wherein both the first and the second single yarn include the one or more additives, and wherein the one or more additives included with the first single yarn are different from the one or more additives included with the second single yarn.

14. Use of the combination yarn according to any of the preceding claims in the manufacture of a carpet, preferably a tufted carpet.

15. Tufted carpet comprising a pile yarn providing the pile of the carpet, the pile yarn being a combination yarn of any one of claims 1-13.

## Patentansprüche

1. Kombiniertes Garn, das ein erstes Einzelgarn und ein zweites Einzelgarn umfasst;
wobei das erste Einzelgarn und das zweite Einzelgarn miteinander verbunden sind;
wobei das erste Einzelgarn mindestens 60 % Polyethylenterephthalat (PET) umfasst;
wobei das zweite Einzelgarn mindestens 60 % Polytrimethylenterephthalat (PTT) umfasst; und
wobei mindestens ein aus dem ersten Einzelgarn und dem zweiten Einzelgarn ausgewähltes Garn einen oder mehrere Zusatzstoffe enthält, die die Farbstoffaufnahme von Dispersionsfarbstoffen oder Lösungsfarbstoffen derart erhöhen, dass die Farbstärke des mindestens einen aus dem ersten Einzelgarn und dem zweiten Einzelgarn ausgewählten Garns im Vergleich zu demselben ersten Einzelgarn und/oder demselben zweiten Einzelgarn, das den einen oder die mehreren Zusatzstoffe nicht enthält, erhöht ist.

2. Kombiniertes Garn nach Anspruch 1, **dadurch gekennzeichnet, dass** der eine oder die mehreren Zusatzstoffe Polybutylenterephthalat (PBT), mindestens einen Estermodifikator oder Kombinationen davon enthalten.

3. Kombiniertes Garn nach Anspruch 2, **dadurch gekennzeichnet, dass** der Estermodifikator das Folgende umfasst:
ein Copolymer, das durch Polymerisation einer Mischung erzielt wird, die Terephthalsäure oder deren Ester, mindestens ein Monomer auf Dicarbonsäurebasis und mindestens ein Monomer auf Diolbasis umfasst,
wobei das mindestens eine Monomer auf Dicarbonsäurebasis ausgewählt ist aus einer aliphatischen und/oder aromatischen Säure, aus Isophthalsäure, 2,6-Naphthalindicarbonsäure, 3,4'-Diphenyletherdicarbonsäure, Hexahydrophthalsäure, 2,7-Naphthalindicarbonsäure, Phthalsäure, 4,4'-Methylenbis(benzoesäure), Oxalsäure, Malonsäure, Bernsteinsäure, Methylbernsteinsäure, Glutarsäure, Adipinsäure, 3-Methyladipinsäure, Pimelinsäure, Suberinsäure, Azelainsäure, Sebacinsäure, 1,11-Undecandicarbonsäure, 1,10-Dodecandicarbonsäure, Undecandicarbonsäure, 1,12-Dodecandicarbonsäure, Hexadecandicarbonsäure, Docosandicarbonsäure, Tetracosandicarbonsäure, 1,4-Cyclohexandicarbonsäure, 1,3-Cyclohexandicarbonsäure, 1,2-Cyclohexandiessigsäure, Fumarsäure, Maleinsäure oder Kombinationen davon, oder aus Bernsteinsäure, Glutarsäure, Adipinsäure, Sebacinsäure oder Kombinationen davon; oder wobei das mindestens eine Monomer auf Dicarbonsäurebasis Adipinsäure ist; oder
wobei der Estermodifikator ein Copolymer, das durch Polymerisation einer Mischung erzielt wird, die Terephthalsäure oder deren Ester, mindestens ein Monomer auf Diolbasis und mindestens ein Polyalkylenglykol umfasst.

4. Kombiniertes Garn nach Anspruch 2, **dadurch gekennzeichnet, dass** der Estermodifikator aus der Gruppe ausgewählt ist, die aus ortho-Phthalsäure, Isophthalsäure oder aus Estern davon besteht.

5. Kombiniertes Garn nach einem der vorstehenden Ansprüche, **dadurch gekennzeichnet, dass** das erste Einzelgarn mindestens 75 % PET umfasst, und/oder dass das zweite Einzelgarn mindestens 75 % PTT umfasst.

6. Kombiniertes Garn nach einem der vorstehenden Ansprüche, **dadurch gekennzeichnet, dass** das erste Einzelgarn und/oder das zweite Einzelgarn ein gebauschtes Endlosfilament für Teppichböden ist.

7. Kombiniertes Garn nach einem der vorstehenden Ansprüche, **dadurch gekennzeichnet, dass** das Gewichtsverhältnis von PET zu PTT in dem kombinierten Garn 1:1 bis 1:4 beträgt.

8. Kombiniertes Garn nach einem der vorstehenden Ansprüche 1-7, **dadurch gekennzeichnet, dass** das erste Einzelgarn den einen oder die mehreren Zusatzstoffe enthält;
wobei die Farbstärke des ersten Einzelgarns innerhalb von 20 % oder innerhalb von 10 % der Farbstärke des zweiten Einzelgarns liegt, wenn beide Garne den gleichen Färbebedingungen unterworfen werden;
wobei die Farbstärke des mindestens einen aus dem ersten Einzelgarn und dem zweiten Einzelgarn ausgewählten Garns durch einen K/S-Wert ausgedrückt wird;
wobei K die Absorption und S die Streuung des Materials darstellt;
wobei der oben genannte Wert durch ein Spektralphotometer bestimmt wird und/oder aus der Kubelka-Munk-Formel berechnet wird.

9. Kombiniertes Garn nach einem der Ansprüche 1-8,
wobei das erste Einzelgarn mindestens 75 % PET und einen Zusatzstoff umfasst, der mindestens einen Estermodifikator enthält;
wobei das zweite Einzelgarn mindestens 75 % PTT umfasst, und keinen Zusatzstoff enthält, der die Farbstoffaufnahme von Dispersionsfarbstoffen oder Lösungsfarbstoffen erhöht; und
wobei die Farbstärke des ersten Einzelgarns innerhalb von 10 % der Farbstärke des zweiten Einzelgarns liegt, wenn beide Garne den gleichen Färbebedingungen unterworfen werden;
wobei die Farbstärke des mindestens einen aus dem ersten Einzelgarn und dem zweiten Einzelgarn ausgewählten Garns durch einen K/S-Wert ausgedrückt wird;
wobei K die Absorption und S die Streuung des Materials darstellt;
wobei der oben genannte Wert durch ein Spektralphotometer bestimmt wird und/oder aus der Kubelka-Munk-Formel berechnet wird.

10. Kombiniertes Garn nach einem der vorstehenden Ansprüche 1-7, **dadurch gekennzeichnet, dass** das zweite Einzelgarn den einen oder die mehreren Zusatzstoffe enthält,
wobei die Farbstärke des zweiten Einzelgarns um mindestens 10 % oder um mindestens 20 % größer ist als die Farbstärke des ersten Einzelgarns, wenn beide Garne den gleichen Färbebedingungen unterworfen werden;
wobei die Farbstärke des mindestens einen aus dem ersten Einzelgarn und dem zweiten Einzelgarn ausgewählten Garns durch einen K/S-Wert ausgedrückt wird;
wobei K die Absorption und S die Streuung des Materials darstellt;
wobei der oben genannte Wert durch ein Spektralphotometer bestimmt wird und/oder aus der Kubelka-Munk-Formel berechnet wird.

11. Kombiniertes Garn nach einem der vorstehenden Ansprüche 1-7 oder 10,
wobei das erste Einzelgarn mindestens 75 % PET umfasst, und keinen Zusatzstoff enthält, der die Farbstoffaufnahme von Dispersionsfarbstoffen oder Lösungsfarbstoffen erhöht;
wobei das zweite Einzelgarn mindestens 75 % PTT und einen Zusatzstoff umfasst, der PBT und mindestens einen Estermodifikator enthält, und
wobei die Farbstärke des zweiten Einzelgarns um mindestens 20 % größer ist als die Farbstärke des ersten Einzelgarns, wenn beide Garne den gleichen Färbebedingungen unterworfen werden;
wobei die Farbstärke des mindestens einen aus dem ersten Einzelgarn und dem zweiten Einzelgarn ausgewählten Garns durch einen K/S-Wert ausgedrückt wird;
wobei K die Absorption und S die Streuung des Materials darstellt;
wobei der oben genannte Wert durch ein Spektralphotometer bestimmt wird und/oder aus der Kubelka-Munk-Formel berechnet wird.

12. Kombiniertes Garn nach einem der vorstehenden Ansprüche 1-7 oder 10,
wobei das erste Einzelgarn mindestens 75 % PET umfasst;
wobei das zweite Einzelgarn mindestens 95 % PTT umfasst;
wobei sowohl das erste Einzelgarn als auch das zweite Einzelgarn weiterhin einen Zusatzstoff umfassen, der PBT, mindestens einen Estermodifikator oder Kombinationen davon enthält; und
wobei die Farbstärke des zweiten Einzelgarns um mindestens 20 % größer ist als die Farbstärke des ersten Einzelgarns, wenn beide Garne den gleichen Färbebedingungen unterworfen werden;
wobei die Farbstärke des mindestens einen aus dem ersten Einzelgarn und dem zweiten Einzelgarn ausgewählten Garns durch einen K/S-Wert ausgedrückt wird;
wobei K die Absorption und S die Streuung des Materials darstellt;
wobei der oben genannte Wert durch ein Spektralphotometer bestimmt wird und/oder aus der Kubelka-Munk-Formel berechnet wird.

13. Kombiniertes Garn nach einem der vorstehenden Ansprüche, ausgenommen Ansprüche 9 und 11,
wobei sowohl das erste Einzelgarn als auch das zweite Einzelgarn den einen oder die mehreren Zusatzstoffe enthalten; und
wobei die einen oder mehreren Zusatzstoffe, die in dem ersten einzelnen Garn enthalten sind, sich von den einen oder mehreren Zusatzstoffen unterscheiden, die in dem zweiten einzelnen Garn enthalten sind.

14. Verwendung des kombinierten Garns nach einem der vorstehenden Ansprüche, zur Herstellung eines Teppichs, vorzugsweise eines getufteten Teppichs.

15. Getufteter Teppich, der ein Florgarn umfasst, das den Flor des Teppichs bildet, wobei das Florgarn ein kombiniertes Garn nach einem der Ansprüche 1 bis 13 ist.

## Revendications

1. Fil issu d'une combinaison qui comprend un premier fil individuel et un deuxième fil individuel ;
dans lequel le premier fil individuel et le deuxième fil individuel sont reliés l'un à l'autre ;
dans lequel le premier fil individuel comprend au moins 60 % de polyéthylène téréphtalate (PET) ;
dans lequel le deuxième fil individuel comprend au moins 60 % de polytriméthylène téréphtalate (PTT) ; et
dans lequel au moins un fil choisi parmi le premier fil individuel et le deuxième fil individuel englobe un ou plusieurs additifs qui augmentent l'absorption de colorant de colorants dispersés ou de colorants en solution, d'une manière telle que l'intensité de la couleur dudit au moins un fil choisi parmi le premier fil individuel et le deuxième fil individuel est augmentée par comparaison à celle du même premier fil individuel et/ou du même deuxième fil individuel qui n'englobe(nt) pas lesdits un ou plusieurs additifs.

2. Fil issu d'une combinaison selon la revendication 1, **caractérisé en ce que** lesdits un ou plusieurs additifs englobent du polybutylène téréphtalate (PBT), au moins un modificateur de type ester, ou leurs combinaisons.

3. Fil issu d'une combinaison selon la revendication 2, **caractérisé en ce que** le modificateur de type ester comprend un copolymère que l'on obtient par polymérisation d'un mélange qui comprend de l'acide téréphtalique ou ses esters, au moins un monomère à base d'acide dicarboxylique, et au moins un monomère à base de diol ;
dans lequel ledit au moins un monomère à base d'acide dicarboxylique est choisi à partir d'un acide aliphatique et/ou aromatique, à partir de l'acide isophtalique, de l'acide 2,6-naphtalène dicarboxylique, de l'acide 3,4'-diphényl éther dicarboxylique, de l'acide hexahydrophtalique, de l'acide 2,7-naphtalène dicarboxylique, de l'acide phtalique, de l'acide 4,4'-méthylène bis(benzoïque), de l'acide oxalique, de l'acide malonique, de l'acide succinique, de l'acide méthyl succinique, de l'acide glutarique, de l'acide adipique, de l'acide 3-méthyl adipique, de l'acide pimélique, de l'acide subérique, de l'acide azélaïque, de l'acide sébacique, de l'acide 1,11-undécane dicarboxylique, de l'acide 1,10-décane dicarboxylique, de l'acide undécane dioïque, de l'acide 1,12-dodécane dicarboxylique, de l'acide hexadécane dioïque, de l'acide docosane dioïque, de l'acide tétracosane dioïque, de l'acide 1,4-cyclohexane dicarboxylique, de l'acide 1,3-cyclohexane dicarboxylique, de l'acide 1,2-cyclohexane diacétique, de l'acide fumarique, de l'acide maléique, ou de leurs combinaisons, ou bien de l'acide succinique, de l'acide glutarique, de l'acide adipique, de l'acide sébacique, ou de leurs combinaisons ; ou dans lequel ledit au moins un monomère à base d'acide dicarboxylique est l'acide adipique ; ou
le modificateur de type ester comprend un copolymère que l'on obtient par polymérisation d'un mélange qui comprend de l'acide téréphtalique ou ses esters, au moins un monomère base de diol, et au moins un polyalkylène glycol.

4. Fil issu d'une combinaison selon la revendication 2, **caractérisé en ce que** le modificateur de type ester est choisi à partir du groupe constitué par l'acide orthophtalique, l'acide isophtalique, ou leurs esters.

5. Fil issu d'une combinaison selon l'une quelconque des revendications précédentes, **caractérisé en ce que** le premier fil individuel comprend au moins 75 % de PET, et/ou **en ce que** le deuxième fil individuel comprend au moins 75 % de PTT.

6. Fil issu d'une combinaison selon l'une quelconque des revendications précédentes, **caractérisé en ce que** le premier fil individuel et/ou le deuxième fil individuel représente(nt) un fil sous la forme d'un filament continu gonflant pour moquette.

7. Fil issu d'une combinaison selon l'une quelconque des revendications précédentes, **caractérisé en ce que** le rapport pondéral du PET au PTT dans le fil issu d'une combinaison s'élève de 1 : 1 à 1 : 4.

8. Fil issu d'une combinaison selon l'une quelconque des revendications 1 à 7, **caractérisé en ce que** le premier fil individuel englobe lesdits un ou plusieurs additifs ;
dans lequel l'intensité de la couleur du premier fil individuel se situe au sein de 20 % ou au sein de 10 % de l'intensité de la couleur du deuxième fil individuel lorsque les deux fils sont soumis aux mêmes conditions de teinture ;
dans lequel l'intensité de la couleur dudit au moins un fil choisi parmi le premier fil individuel et le deuxième fil individuel est exprimée par une valeur K/S ;
dans lequel K représente l'absorption et S représente la diffusion de la matière ;
dans lequel ladite valeur est déterminée par l'intermédiaire d'un spectrophotomètre et/ou est calculée à partir de la formule de Kubelka-Munk.

9. Fil issu d'une combinaison selon l'une quelconque des revendications 1 à 8,
dans lequel le premier fil individuel comprend au moins 75 % de PET et un additif qui englobe au moins un modificateur de type ester ;
dans lequel le deuxième fil individuel comprend au moins 75 % de PTT et n'englobe aucun additif qui augmente l'absorption de colorant de colorants dispersés ou de colorants en solution ; et
dans lequel l'intensité de la couleur du premier fil individuel se situe au sein de 10 % de l'intensité de la couleur du deuxième fil individuel lorsque les deux fils sont soumis aux mêmes conditions de teinture ;
dans lequel l'intensité de la couleur dudit au moins un fil choisi parmi le premier fil individuel et le deuxième fil individuel est exprimée par une valeur K/S dans lequel K représente l'absorption et S représente la diffusion de la matière ;
dans lequel ladite valeur est déterminée par l'intermédiaire d'un spectrophotomètre et/ou est calculée à partir de la formule de Kubelka-Munk.

10. Fil issu d'une combinaison selon l'une quelconque des revendications 1 à 7 précédentes, **caractérisé en ce que** le deuxième fil individuel englobe lesdits un ou plusieurs additifs ;
dans lequel l'intensité de la couleur du deuxième fil individuel est supérieure à l'intensité de la couleur du premier fil individuel à raison d'au moins 10 % ou à raison d'au moins 20 %, lorsque les deux fils sont soumis aux mêmes conditions de teinture ;
dans lequel l'intensité de la couleur dudit au moins un fil choisi parmi le premier fil individuel et le deuxième fil individuel est exprimée par une valeur K/S ;
dans lequel K représente l'absorption et S représente la diffusion de la matière ;
dans lequel ladite valeur est déterminée par l'intermédiaire d'un spectrophotomètre et/ou est calculée à partir de la formule de Kubelka-Munk.

11. Fil issu d'une combinaison selon l'une quelconque des revendications 1 à 7 ou 10,
dans lequel le premier fil individuel comprend au moins 75 % de PET et n'englobe aucun additif qui augmente l'absorption de colorant de colorants dispersés ou de colorants en solution ;
dans lequel le deuxième fil individuel comprend au moins 75 % de PTT et un additif qui englobe du PBT et au moins un modificateur de type ester ; et
dans lequel l'intensité de la couleur du deuxième fil individuel est supérieure à l'intensité de la couleur du premier fil individuel à raison d'au moins 20 %, lorsque les deux fils sont soumis aux mêmes conditions de teinture ;
dans lequel l'intensité de la couleur dudit au moins un fil choisi parmi le premier fil individuel et le deuxième fil individuel est exprimée par une valeur K/S ;
dans lequel K représente l'absorption et S représente la diffusion de la matière ;
dans lequel ladite valeur est déterminée par l'intermédiaire d'un spectrophotomètre et/ou est calculée à partir de la formule de Kubelka-Munk.

12. Fil issu d'une combinaison selon l'une quelconque des revendications 1 à 7 ou 10,
dans lequel le premier fil individuel comprend au moins 75 % de PET ;
dans lequel le deuxième fil individuel comprend au moins 75 % de PTT ;
dans lequel à la fois le premier fil individuel et le deuxième fil individuel comprennent en outre un additif qui englobe du PBT, au moins un modificateur de type ester, ou leurs combinaisons ; et
dans lequel l'intensité de la couleur du deuxième fil individuel est supérieure à l'intensité de la couleur du premier fil individuel à raison d'au moins 20 %, lorsque les deux fils sont soumis aux mêmes conditions de teinture ;
dans lequel l'intensité de la couleur dudit au moins un fil choisi parmi le premier fil individuel et le deuxième fil individuel est exprimée par une valeur K/S ;
dans lequel K représente l'absorption et S représente la diffusion de la matière ;
dans lequel ladite valeur est déterminée par l'intermédiaire d'un spectrophotomètre et/ou est calculée à partir de la formule de Kubelka-Munk.

13. Fil issu d'une combinaison selon l'une quelconque des revendications précédentes, à l'exclusion des revendications 9 et 11,
dans lequel à la fois le premier et le deuxième fil individuel englobent les dits un ou plusieurs additifs ; et
dans lequel lesdits un ou plusieurs additifs inclus dans le premier fil individuel sont différents desdits un ou plusieurs additifs inclus dans le deuxième fil individuel.

14. Utilisation du fil issu d'une combinaison selon l'une quelconque des revendications précédentes, dans la confection d'un tapis, de préférence d'une moquette tuftée.

15. Moquette tuftée qui comprend un fil de poil qui procure les poils du tapis ; dans laquelle le fil de poil représente un fil issu d'une combinaison selon l'une quelconque des revendications 1 à 13.
